

Dec. 30, 1958

W. D. WARINNER

2,866,728

DRY MANGANOUS PHOSPHATE COMPOUNDS

Filed April 30, 1956

2 Sheets-Sheet 1

FIG. 1.



INVENTOR

WARREN D. WARINNER

BY *Cameron, Kerkam & Sutton*

ATTORNEYS

Dec. 30, 1958

W. D. WARINNER

2,866,728

## DRY MANGANOUS PHOSPHATE COMPOUNDS

Filed April 30, 1956

2 Sheets-Sheet 2



WARREN D. WARINNER

BY  
Cameron, Kerkam & Sutton  
ATTORNEYS

# United States Patent Office

2,866,728

Patented Dec. 30, 1958

1

2,866,728

## DRY MANGANOUS PHOSPHATE COMPOUNDS

Warren D. Warinner, College Park, Ga., assignor to Tennessee Corporation, New York, N. Y., a corporation of New York

Application April 30, 1956, Serial No. 581,586

7 Claims. (Cl. 148—6.15)

This invention relates to novel dry substantially completely water-soluble manganous phosphate compounds and more particularly to such compounds comprising manganous oxide, phosphorous pentoxide and water in the molar proportions comparable to the composition of manganous dihydrogen orthophosphate on and within which is condensed anhydrous orthophosphoric acid as the acid of crystallization, there being from one-half mole to one mole of orthophosphoric acid per mole of manganous dihydrophosphate and one-half to two and one-half moles of water of crystallization. More particularly still this invention relates to such dry manganous phosphate solid compounds which when dissolved in water will constitute a bath for applying manganous phosphate coatings on metallic surfaces with minimum loss of manganese by hydrolysis when the bath is raised to operating temperatures.

I have found that the dry manganous phosphate compounds of the present invention can not be prepared by fractional crystallization and must be prepared by concentration of a solution containing proper proportions of MnO and P<sub>2</sub>O<sub>5</sub> under conditions which will maintain the manganese in reduced state. The solubility of these compounds is obtained by having a minimum of one-quarter mole of water of crystallization and if the compounds are to be dry within the concept of the present invention the maximum of two and one-half moles of water of crystallization is required.

It has heretofore been proposed to coat metal surfaces with adherent insoluble manganese phosphate films by dipping or by otherwise treating the metal surfaces with manganese in solution. Solutions of manganese in phosphoric acid are known in the art, for example, manganous dihydrophosphate dihydrate. Studies of the systems MnO—P<sub>2</sub>O<sub>5</sub>—H<sub>2</sub>O have been published by M. Amadori, Atti. ist. Venito, 81, 603—17 (1921—22); in the article by Grube and Staesche, Z. physik. Chem., 130, 572—583 (1927); and in the article by Taperova and Isaeva, J. Applied Chem. (USSR) 22, 342—53 (1949). United States patents have issued in this field including Willard No. 1,660,661; Green No. 1,651,694; Booth No. 2,031,557; and MacIntyre No. 2,093,461.

The dry manganous compounds known to the prior art are discussed in these articles and patents have certain undesirable characteristics, the most important of which is either excessive loss of manganese and phosphoric acid from the coating solution by hydrolysis which takes place both in the preparation of the bath and in reconstitution of the bath after use or the retention of excessive amounts of highly acidic mother liquor by the crystals. Fractional crystallization is required to prepare certain of these prior art compounds and the limitations imposed by this procedure results in greater expense and undesirable properties in the compounds prepared.

It is accordingly an object of the present invention to provide novel dry manganous phosphate compounds

2

suitable for the preparation of manganous phosphate coating baths.

Another object is to provide such novel compounds which exhibit negligible loss due to hydrolysis when used in the preparation and reconstitution of coating baths.

Another object is to provide such novel compounds which are substantially completely water-soluble.

Another object is to provide such novel compounds containing available phosphoric acid to maintain a balanced solution in the coating bath.

Another object is to provide such novel compounds having a higher phosphoric acid ratio to manganese than in manganous compounds now in use.

Another object is to provide such novel dry manganous phosphate compounds which, when in solution, will coat metals more uniformly with a thicker coat of manganese phosphate requiring less of the compound to reconstitute the solution after use and which will yield more manganese phosphate as the coating material.

Another object is to provide such novel compounds which have ratios of manganese to phosphoric acid heretofore available only in solutions.

Another object is to provide such novel compounds which may be adjusted in composition to suit a variety of requirements.

Another object is to provide orthophosphoric acid in a non-liquid readily transportable form.

Other and further objects of the present invention will appear from the following description of illustrative embodiments thereof.

I have found that the novel dry manganous phosphate compounds of this invention, having the physical characteristics and advantages described in these objects, have a MnO to P<sub>2</sub>O<sub>5</sub> to H<sub>2</sub>O percentage ratio of approximately 23.3—18.0% MnO; 60.7—51.6% P<sub>2</sub>O<sub>5</sub>; and 28.1—18.7% H<sub>2</sub>O and have a molar ratio of one-half to one mole of orthophosphoric acid per mole of manganous dihydrophosphate and have from one-half to two and one-half moles of water of crystallization. It is therefore apparent that a family of dry manganous phosphate compounds come within the purview of the present inventive concept and that the illustrative embodiments thereof discussed below can in no way be construed as defining or limiting the invention. Reference should therefore be had to the appended claims to determine the scope of the present inventive concept.

The dry manganous phosphate compounds of the present invention may be identified graphically by composition and in the accompanying drawings Fig. 1 is a solubility-isotherm-phase diagram for MnO—P<sub>2</sub>O<sub>5</sub>—H<sub>2</sub>O where the percentage of water is inferred as the difference between 100% and the sum of the percentages of MnO and P<sub>2</sub>O<sub>5</sub> at 25° C., the range of the compounds of the present invention being shown in the area a, b, c, d; and

Fig. 2 is an enlarged detail of a portion of Fig. 1 showing the range of the compounds of the present invention and showing representative compounds within the area of the present invention.

The dry manganous phosphate compounds of the present invention are prepared without requiring fractional crystallization by the addition of a slurry of manganous ion donor to a concentrated solution of phosphoric acid containing sufficient hydrogen peroxide to assure maintenance of the manganous state. No external heat need be applied to the reaction and, upon completion of the reaction, the resultant liquor may be clarified if necessary and then dehydrated as rapidly as possible to the desired degree of dehydration.

More particularly, these novel dry manganous phosphate compounds are preferably prepared by adding either a slurry of manganous carbonate or dry man-

ganous carbonate to phosphoric acid starting at ambient temperatures and applying no external heat during the reaction. Suitable manganous phosphate solutions are assured when a small amount of  $H_2O_2$  is added to the phosphoric acid before the manganous carbonate is added to the acid. About .6 lb.  $H_2O_2$  per 100 lbs. of manganese assures proper control of the reaction and the production of the desired manganous phosphate solutions. Any excess  $H_2O_2$  is driven off during subsequent concentration of the solution at about 60° C. The use of  $H_2O_2$  in a reaction of this type is discussed in British Patent No. 447,918 granted in 1936.

It is highly desirable to avoid the precipitation of crystalline material from the initial liquors previous to the starting of evaporation for practical as well as in British Patent No. 447,918 granted in 1936.

of insoluble pyrophosphates and/or metaphosphates appears to be more a function of time than of temperature, generally occurring during the transition from the hemihydrate to the anhydrous state. Drying temperatures up to 260° F. are preferred.

The use of manganous carbonate is preferred in forming the original slurry as the resulting manganous phosphate solution does not require filtering and impurities are not introduced into the solution as is the case when other sources of manganese are used.

The dry manganous phosphate compounds shown at points *a*, *b*, *c* and *d* of Figs. 1 and 2, defining the limits of the family of compounds of the present invention, are made by the procedures described above and have compositions as described in the following table:

TABLE I

| Sample Point | Composition |             |                  |                | Weight Ratios |              |               |             |              |               |
|--------------|-------------|-------------|------------------|----------------|---------------|--------------|---------------|-------------|--------------|---------------|
|              | Percent Mn  | Percent MnO | Percent $P_2O_5$ | Percent $H_2O$ | $P_2O_5/Mn$   | $P_2O_5/MnO$ | $P_2O_5/H_2O$ | $Mn/P_2O_5$ | $MnO/P_2O_5$ | $H_2O/P_2O_5$ |
| <i>a</i>     | 15.7        | 20.4        | 51.6             | 28.0           | 3.287         | 2.529        | 1.843         | 0.304       | 0.395        | 0.543         |
| <i>b</i>     | 17.9        | 23.3        | 57.7             | 19.0           | 3.224         | 2.476        | 3.037         | 0.310       | 0.404        | 0.392         |
| <i>c</i>     | 15.84       | 20.46       | 60.7             | 18.8           | 3.832         | 2.967        | 3.229         | 0.261       | 0.337        | 0.309         |
| <i>d</i>     | 13.9        | 18.0        | 53.9             | 28.1           | 3.878         | 2.094        | 1.918         | 0.258       | 0.334        | 0.521         |

as technical reasons and I have found that the best results are obtained by liming the maximum concentration of the initial liquors to between 9.6% and 10.8% MnO and 29.0% and 27.5%  $P_2O_5$  by weight; this practice defers the appearance of crystals during evaporation until a considerable amount of concentration has been realized and promotes the formation of very fine crystals which subsequently recrystallize to the desired compositions.

After the desired manganous phosphate solution is obtained approximately two-thirds of the excess water is removed to form a slurry and the final dehydration of the thickened slurry should be accomplished as quickly as possible to avoid the formation of pyrophosphates or the solution may be dehydrated in one step by other methods such as spray drying. The formation

The compounds identified at points *a*, *b*, *c* and *d* in Figs. 1 and 2 and as described in Table I are substantially completely soluble in cold water; they do not hydrolyze; and they have the desired physical characteristics that allow dry packaging without agglomeration. These compounds also withstand pressure without permanent coalescence.

Various dry manganous phosphate compounds within the limits defined by points *a*, *b*, *c* and *d* of Figs. 1 and 2 and having the desired characteristics described above with respect to the compounds of Table I are shown and described in the following tables which compare these compounds with known compounds, the illustrative compounds of the present invention being identified by numerals 10, 11, 12, 13 and 14:

TABLE II

| Manganous Phosphate Compound                  | Solid Materials Used |      |          |                         |        | Gms. Solids per Liter | Initial Solution    |      |          | After Digesting |      |       | Eff. of Solids vs. Alc. Wash. Dihydro. |      |       |     |       |       |       |
|-----------------------------------------------|----------------------|------|----------|-------------------------|--------|-----------------------|---------------------|------|----------|-----------------|------|-------|----------------------------------------|------|-------|-----|-------|-------|-------|
|                                               | Composition, Percent |      |          | Wt. ratio, $P_2O_5/MnO$ | Actual |                       | Composition, Gm./L. |      |          | Pointage        |      |       |                                        |      |       |     |       |       |       |
|                                               | Mn                   | MnO  | $P_2O_5$ |                         |        |                       | Mn                  | MnO  | $P_2O_5$ | pH              | Free | Total | pH                                     | Free | Total |     |       |       |       |
| 10.                                           | 16.6                 | 21.4 | 54.0     | 3.254                   | 3.230  | 20                    | 3.32                | 4.28 | 10.8     | 2.53            | 2.6  | 22.0  | 2.47                                   | 2.8  | 21.8  | 7.8 | 0.910 | 0.806 | 124.1 |
| 11.                                           | 16.5                 | 21.3 | 55.5     | 3.364                   | 3.390  | 20                    | 3.30                | 4.26 | 11.1     | 2.53            | 2.6  | 22.8  | 2.54                                   | 2.9  | 22.8  | 7.9 | 0.876 | 0.775 | 129.0 |
| 12.                                           | 15.9                 | 20.5 | 66.5     | 3.500                   | 3.554  | 20                    | 3.18                | 4.10 | 11.3     | 2.38            | 4.0  | 23.5  | 3.35                                   | 3.6  | 23.5  | 6.5 | 0.851 | 0.753 | 132.8 |
| 13.                                           | 14.5                 | 18.8 | 56.3     | 3.888                   | 3.877  | 25.6                  | 3.72                | 4.82 | 14.4     | 2.32            | 4.5  | 30.4  | 2.40                                   | 5.4  | 30.4  | 5.6 | 0.842 | 0.745 | 134.2 |
| 14.                                           | 17.2                 | 22.2 | 58.5     | 3.340                   | 3.390  | 20                    | 3.44                | 4.44 | 11.7     | 2.48            | 2.7  | 23.5  | 2.53                                   | 2.7  | 23.8  | 8.8 | 0.840 | 0.743 | 134.6 |
| Centrif. Dihydro-Alc. Wash. Dihydro phosphate | 18.2                 | 23.5 | 49.2     | 2.702                   | 2.584  | 33.7                  | 6.25                | 7.90 | 16.6     | 3.30            | 0.2  | 30.3  | 2.39                                   | 4.6  | 29.1  | 6.3 | 1.147 | 1.010 | 99.0  |
|                                               | 18.9                 | 24.4 | 49.5     | 2.616                   | 2.584  | 20.0                  | 3.78                | 4.88 | 9.9      | 3.70            | 0.0  | 18.4  | 2.36                                   | 2.9  | 17.7  | 6.1 | 1.130 | 1.000 | 100.0 |

Composition #10 represents substantially  $\frac{1}{2} H_2PO_4 \cdot Mn(H_2PO_4)_2 \cdot 1\frac{1}{2} H_2O$ .

Composition #11 represents substantially  $\frac{1}{2} H_2PO_4 \cdot Mn(H_2PO_4)_2 \cdot 1\frac{1}{2} H_2O$ .

Composition #12 represents substantially  $\frac{1}{2} H_2PO_4 \cdot Mn(H_2PO_4)_2 \cdot 1\frac{1}{2} H_2O$ .

Composition #13 represents substantially  $\frac{1}{2} H_2PO_4 \cdot Mn(H_2PO_4)_2 \cdot 1\frac{1}{2} H_2O$ .

Composition #14 represents substantially  $\frac{1}{2} H_2PO_4 \cdot Mn(H_2PO_4)_2 \cdot 1\frac{1}{2} H_2O$ .

"Centrif. Dihydro." =  $Mn(H_2PO_4)_2 \cdot 2H_2O$  crystals prepared by fractional crystallization per existing patent disclosures and centrifuged to separate from major part of mother liquor.

"Alc. Washed Dihydrophosphate" = "Centrif. Dihydro." which was washed carefully with ethyl alcohol to remove the adsorbed mother liquor.

"After Digesting" = the initial solutions were maintained at 200-208° F. for 4-5 hours.

"Solids" in the headings of the columns refers to the compounds cited in column #1.

TABLE II-a  
Comparison of losses due to hydrolysis

| Manganous Phosphate Compound         | Gms. Solids Ppt'd by Digestion | Percent of Original Wt. of Dissolved Solids | Av. Comp. of Ppt. |                               | Gms. Ppt'd by Digestion |                               | Percent of Loss from Digestion |                               |
|--------------------------------------|--------------------------------|---------------------------------------------|-------------------|-------------------------------|-------------------------|-------------------------------|--------------------------------|-------------------------------|
|                                      |                                |                                             | Mn                | P <sub>2</sub> O <sub>5</sub> | Mn                      | P <sub>2</sub> O <sub>5</sub> | Mn                             | P <sub>2</sub> O <sub>5</sub> |
| 10                                   | 0.81                           | 4.07                                        | 37.1              | 38.4                          | 0.30                    | 0.31                          | 9.0                            | 2.9                           |
| 11                                   | 0.13                           | 0.65                                        | 37.1              | 38.4                          | 0.05                    | 0.05                          | 1.5                            | 0.4                           |
| 12                                   | 0                              | 0                                           | 0                 | 0                             | 0                       | 0                             | 0                              | 0                             |
| 13                                   | 0                              | 0                                           | 0                 | 0                             | 0                       | 0                             | 0                              | 0                             |
| 14                                   | 0                              | 0                                           | 0                 | 0                             | 0                       | 0                             | 0                              | 0                             |
| Centrif. Dihydro-Alc. Wash. Di-hydro | 5.56                           | 16.5                                        | 37.1              | 38.4                          | 2.07                    | 2.14                          | 33.1                           | 12.9                          |
| or                                   | 3.53                           | 17.6                                        | 37.1              | 38.4                          | 1.31                    | 1.35                          | 39.3                           | 13.7                          |

This table tabulates the losses found when the cited illustrative solutions were heated to the operating temperature range.

Recognizing the limits of accuracy of conventional analytical methods for the determination of manganese and phosphorus, point "a," Fig. 2, is substantially



or



ity of the novel dry manganous phosphate compounds of the present invention is also illustrated with respect to free acid and total acid; with respect to pH as compared to known compounds; with respect to manganese concentration at various temperatures as compared to known compounds; and with respect to P<sub>2</sub>O<sub>5</sub> concentrations at various temperatures.

The following table illustrates the weight ratios of the components of the novel dry manganous phosphate compounds of this invention:

TABLE III

Weight ratios

| Empirical Formula                                                                                            | P <sub>2</sub> O <sub>5</sub><br>Mn | P <sub>2</sub> O <sub>5</sub><br>MnO | P <sub>2</sub> O <sub>5</sub><br>H <sub>2</sub> O | Mn<br>P <sub>2</sub> O <sub>5</sub> | MnO<br>P <sub>2</sub> O <sub>5</sub> | H <sub>2</sub> O<br>P <sub>2</sub> O <sub>5</sub> |
|--------------------------------------------------------------------------------------------------------------|-------------------------------------|--------------------------------------|---------------------------------------------------|-------------------------------------|--------------------------------------|---------------------------------------------------|
| Mn(H <sub>2</sub> PO <sub>4</sub> ) <sub>2</sub> · H <sub>3</sub> PO <sub>4</sub> · 1/4 H <sub>2</sub> O     | 3.876                               | 3.00                                 | 3.15                                              | 0.2580                              | 0.333                                | 0.317                                             |
| Mn(H <sub>2</sub> PO <sub>4</sub> ) <sub>2</sub> · H <sub>3</sub> PO <sub>4</sub> · 1/2 H <sub>2</sub> O     | 3.876                               | 3.00                                 | 2.95                                              | 0.2580                              | 0.333                                | 0.339                                             |
| Mn(H <sub>2</sub> PO <sub>4</sub> ) <sub>2</sub> · H <sub>3</sub> PO <sub>4</sub> · 2/3 H <sub>2</sub> O     | 3.876                               | 3.00                                 | 1.97                                              | 0.2580                              | 0.333                                | 0.508                                             |
| Mn(H <sub>2</sub> PO <sub>4</sub> ) <sub>2</sub> · 3/4 H <sub>3</sub> PO <sub>4</sub> · 1/2 H <sub>2</sub> O | 3.554                               | 2.752                                | 2.99                                              | 0.2814                              | 0.3633                               | 0.334                                             |
| Mn(H <sub>2</sub> PO <sub>4</sub> ) <sub>2</sub> · 3/4 H <sub>3</sub> PO <sub>4</sub> · 2/3 H <sub>2</sub> O | 3.554                               | 2.752                                | 1.92                                              | 0.2814                              | 0.3633                               | 0.523                                             |
| Mn(H <sub>2</sub> PO <sub>4</sub> ) <sub>2</sub> · 5/6 H <sub>3</sub> PO <sub>4</sub> · 1/2 H <sub>2</sub> O | 3.390                               | 2.625                                | 3.01                                              | 0.2949                              | 0.3809                               | 0.332                                             |
| Mn(H <sub>2</sub> PO <sub>4</sub> ) <sub>2</sub> · 5/6 H <sub>3</sub> PO <sub>4</sub> · 2/3 H <sub>2</sub> O | 3.390                               | 2.625                                | 1.91                                              | 0.2949                              | 0.3809                               | 0.529                                             |
| Mn(H <sub>2</sub> PO <sub>4</sub> ) <sub>2</sub> · 1/2 H <sub>3</sub> PO <sub>4</sub> · 1/2 H <sub>2</sub> O | 3.230                               | 2.502                                | 3.02                                              | 0.3096                              | 0.3997                               | 0.331                                             |
| Mn(H <sub>2</sub> PO <sub>4</sub> ) <sub>2</sub> · 1/2 H <sub>3</sub> PO <sub>4</sub> · 2/3 H <sub>2</sub> O | 3.230                               | 2.502                                | 1.83                                              | 0.3096                              | 0.3997                               | 0.531                                             |

and can be called "dimanganous henidecahydropentaphosphate pentahydrate," while point "b" is correspondingly the monohydrate. The hydrates of this salt are sufficiently rich in manganese to provide a moderate buffering effect when introduced into coating baths overly rich in acidity.

Point "d," Fig. 2, is substantially



or



and can be named "manganous heptahydrotriorthophosphate hemipentahydrate," while point "c" would be the quarter or tetrahydrate; these compositions are sufficiently rich in phosphoric acid in respect to manganese to supply a moderate amount of excess free acidity which may be desirable and useful where films of rust must be removed concurrently with the deposition of protective coatings. Of particular interest is the composition



shown in Table III, and illustrated by compound 12; these compounds may be written



and may be named "tetramanganous pentacosihydrohen-decaorthophosphate (di- to deca) hydrate;" these compounds dissolve in water to provide the optimum ratio of manganese to phosphoric acid for the preparation and maintenance of manganous phosphate coating baths.

The data set out in Tables II and II-a illustrates the economies available in the use of the compositions of the present invention as compared to prior art manganous compounds, usually Mn(H<sub>2</sub>PO<sub>4</sub>)<sub>2</sub> · 2H<sub>2</sub>O, in the quantities required to produce unit point total acidity. The stabil-

A "thirty point" manganous phosphate solution made from dihydrogen phosphate crystals prepared according to the prior art will hydrolyze to some extent in the cold. When a solution of this phosphate is heated to prepare it for the coating operation a considerable quantity of precipitate is formed which is entirely insoluble and amounts to approximately 31% of the manganese and 12.9% of the P<sub>2</sub>O<sub>5</sub> originally introduced into the bath. Thus the bath undergoes a radical change in character. A "thirty point" solution prepared with a dry manganous phosphate compound of the present invention is completely soluble, does not hydrolyze when heated to prepare the solution as a coating bath and the bath remains clear. As shown in Tables II and II-a, baths ranging between 20 and 25 points also exhibit the same characteristics. In connection with these solutions it is to be understood that the term "point" means the number of milliliters of 0.1 normal sodium hydroxide required to titrate a 10.0 ml. sample of the bath to the phenolphthalein end point. The two solutions are substantially the same chemically after heating but a coating bath can be maintained with less of the compounds of the present invention on a weight basis as compared to the dihydrogen phosphate compounds of the prior art in the approximate ratio of 75 to 100.

After using the baths for identical coating operations it is found that the loss of manganese in the sludge resulting from the operation of the bath employing the manganous phosphate compounds of the present invention is 23% of the loss from the bath employing manganous dihydrogen orthophosphate prepared according to the prior art. The loss of P<sub>2</sub>O<sub>5</sub> in the sludge found in the bath of the present invention is 42% of that lost from the prior art dihydrogen orthophosphate bath. Compar-

ing the weight of sludges formed during the operation of the baths it is found that the bath employing the compounds of the present invention contains a sludge which is 42% by weight, dry basis, of that found in the bath employing the manganous phosphate of the prior art.

The coating baths were conditioned by treating eight successive panels in each bath before the data was collected to obtain the results discussed above. The coatings on the panels from the bath utilizing the manganous phosphate compounds of the present invention are uniform in appearance and in weight for all of the panels throughout all of the cycles while the coatings provided by the bath of manganous dihydrogen orthophosphate prepared in accordance with the prior art deteriorate in quality as the test progresses. It is also found that there is less etching or attack on the surface of the panels being coated by the bath made up from the compounds of the present invention.

After the above solutions had been conditioned by treating the equivalent of 10 square feet of standard test panel surface per gallon, a series of three panels was treated in each bath for one hour per panel and the baths were brought back to a 30 point strength previous to each treatment. All three panels treated in the coating bath prepared from the material of the present invention were uniformly coated, while the coating on the second and third panels treated in the bath prepared from manganous dihydrogen phosphate prepared according to prior art was very inferior to that on the first panel. Table IV summarizes the averaged coating data.

TABLE IV

|                                    | Present Invention Material | Prior Art Dihydrogen Phosphate |
|------------------------------------|----------------------------|--------------------------------|
| Coating wt., mg./ft. <sup>2</sup>  | 3.372                      | 1,656                          |
| Etching loss, mg./ft. <sup>2</sup> | 3.510                      | 3,985                          |
| Free Acid-Points:                  |                            |                                |
| start                              | 5.0                        | 5.1                            |
| finish                             | 3.2                        | 3.3                            |
| Total Pointage:                    |                            | 40                             |
| start                              | 29.8                       | 29.3                           |
| finish                             | 26.1                       | 25.5                           |

Panels coated from baths employing the manganous phosphate compounds of the present invention may be tested by the method described by Andrews et al. in Journal of Applied Chemistry, volume 4, pages 581-595, of November 4, 1954, and the protective properties of the coats may be compared by the "copper spot test" as reported by Akimov et al., USSR Academy of Sciences, Moscow, 1946, page 117. These tests show that manganese phosphate coats obtained from solutions in accordance with the present invention are more uniform than those of the prior art; that more manganese phosphate is available in the solutions for coating and that more manganese phosphate is recovered as useful coating material; and the "copper spot test" shows that panels coated from solutions of the present invention are substantially completely protected.

It should now be apparent that the present invention in every way satisfies the several objectives described above.

Changes in or modifications to the above described illustrative procedures and compounds may now be suggested to those skilled in the art without departing from the present invention. Reference should therefore be

had to the appended claims to determine the scope of the present inventive concept.

What is claimed is:

1. Dry acidulous water soluble manganous phosphate compounds consisting of approximately 18.0-23.3% MnO, approximately 51.6-60.7% P<sub>2</sub>O<sub>5</sub> and approximately 18.7-28.1% H<sub>2</sub>O in molar ratio of from one mole of manganous oxide and from one and one-quarter to one and one-half moles of phosphorous pentoxide and from three and one-quarter to six moles of water of which from one-half to two and one-half moles of water is present as water of crystallization.

2. Dry water soluble acid salts of manganous phosphate compounds consisting of manganous dihydrophosphate containing as the acid of crystallization condensed anhydrous orthophosphoric acid in the ratio of from one-half mole to one mole of orthophosphoric acid per mole of manganous dihydrophosphate and including one-half to two and one-half moles of water of crystallization.

3. Dry water soluble acid salts of manganous phosphate compounds having the empirical formula



and weight ratios P<sub>2</sub>O<sub>5</sub>/Mn=3.876, P<sub>2</sub>O<sub>5</sub>/MnO=3.00 and P<sub>2</sub>O<sub>5</sub>/H<sub>2</sub>O=2.95-1.97.

4. Dry water soluble acid salts of manganous phosphate compounds having the empirical formula



and weight ratios P<sub>2</sub>O<sub>5</sub>/Mn=3.554, P<sub>2</sub>O<sub>5</sub>/MnO=2.752 and P<sub>2</sub>O<sub>5</sub>/H<sub>2</sub>O=2.99-1.92.

5. Dry water soluble acid salts of manganous phosphate compounds having the empirical formula



and weight ratios P<sub>2</sub>O<sub>5</sub>/Mn=3.390, P<sub>2</sub>O<sub>5</sub>/MnO=2.625 and P<sub>2</sub>O<sub>5</sub>/H<sub>2</sub>O=3.01-1.91.

6. Dry water soluble acid salts of manganous phosphate compounds having the empirical formula



and weight ratios P<sub>2</sub>O<sub>5</sub>/Mn=3.230, P<sub>2</sub>O<sub>5</sub>/MnO=2.502 and P<sub>2</sub>O<sub>5</sub>/H<sub>2</sub>O=3.02-1.83.

7. Dry water soluble acid salts of manganous phosphate compounds having an empirical formula



and weight ratios

P<sub>2</sub>O<sub>5</sub>/Mn=3.230-3.876, P<sub>2</sub>O<sub>5</sub>/MnO=2.502-3.0 and P<sub>2</sub>O<sub>5</sub>/H<sub>2</sub>O=3.025-1.829.

#### References Cited in the file of this patent

#### UNITED STATES PATENTS

- 55 2,310,239 Jernstedt Feb. 9, 1943  
 2,516,008 Lum July 18, 1950  
 2,516,139 Mazia July 25, 1950

#### FOREIGN PATENTS

- 60 365,569 Great Britain Printed 1932  
 447,918 Great Britain May 27, 1936

#### OTHER REFERENCES

- Mellor: "Comprehensive Treatise on Inorganic and Theoretical Chemistry," vol. 12, pages 451, 452, published 1932. Copy in Sci. Lib.

UNITED STATES PATENT OFFICE  
Certificate of Correction

Patent No. 2,866,728

December 30, 1958

Warren D. Warinner

It is hereby certified that error appears in the printed specification of the above numbered patent requiring correction and that the said Letters Patent should read as corrected below.

Column 3, line 32, for "liming" read —limiting—; columns 3 and 4, Table II, twelfth column thereof, fourth item under the subheading "Free", for "4.5" read —5.4—; in the footnote at bottom of same page, third line from the last, for "alcoh" read —alcohol—.

Signed and sealed this 28th day of April 1959.

[SEAL]

Attest:

T. B. MORROW,  
*Attesting Officer.*

ROBERT C. WATSON,  
*Commissioner of Patents.*